



US005114326A

## United States Patent [19]

Wüllenweber et al.

[11] Patent Number: 5,114,326

[45] Date of Patent: May 19, 1992

## [54] APPARATUS FOR MANUFACTURING DIAPHRAGMS

[75] Inventors: Heinz Wüllenweber, Frankfurt am Main; Peter Kohl, Neuberg; Herbert Jung, Oberursel, all of Fed. Rep. of Germany; Jürgen Borchardt, Troistorrents, Switzerland; Wolfgang Bickle, Reilingen, Fed. Rep. of Germany; Jürgen Braus, Walldorf, Fed. Rep. of Germany; Hans-Joachim Hiedemann, Cologne, Fed. Rep. of Germany

[73] Assignees: Metallgesellschaft AG, Frankfurt am Main; Kollbenschmidt, Neckarsulm; Jean Hiedemann GmbH & Co. KG, Cologne, all of Fed. Rep. of Germany

[21] Appl. No.: 554,642

[22] Filed: Jul. 17, 1990

## Related U.S. Application Data

[62] Division of Ser. No. 339,747, Apr. 18, 1989, Pat. No. 4,961,901.

## [30] Foreign Application Priority Data

Apr. 23, 1988 [DE] Fed. Rep. of Germany ..... 3813743

[51] Int. Cl.<sup>5</sup> ..... B22F 3/18

[52] U.S. Cl. ..... 425/79; 425/373

[58] Field of Search ..... 425/79, 78, 218, 219, 425/220, 224, 365, 375, 373, 374, 515, 517, 520; 118/256, 19, 242

[56]

## References Cited

## U.S. PATENT DOCUMENTS

|           |         |                 |         |
|-----------|---------|-----------------|---------|
| 1,930,287 | 10/1933 | Short et al.    | 425/79  |
| 2,341,732 | 2/1944  | Marvin          | 425/79  |
| 2,917,821 | 12/1959 | Fritsch         | 425/79  |
| 3,194,858 | 7/1965  | Storchheim      | 425/79  |
| 3,403,999 | 10/1968 | Bliss           | 419/43  |
| 4,172,111 | 10/1979 | Donnelly        | 264/111 |
| 4,325,995 | 4/1982  | Tamura et al.   | 118/242 |
| 4,670,214 | 6/1987  | Magnuson et al. | 264/171 |

## FOREIGN PATENT DOCUMENTS

|         |         |          |        |
|---------|---------|----------|--------|
| 119772  | of 1959 | U.S.S.R. | 425/79 |
| 980962  | 12/1982 | U.S.S.R. | 425/79 |
| 1041214 | 9/1983  | U.S.S.R. | 425/79 |
| 1444081 | 12/1988 | U.S.S.R. | 425/79 |

Primary Examiner—Richard L. Chiesa

Assistant Examiner—W. J. Matney, Jr.

Attorney, Agent, or Firm—Sprung Horn Kramer &amp; Woods

[57]

## ABSTRACT

In an apparatus of manufacturing diaphragms, a layer of a difficultly flowable metal powder is applied to a support, a wire net is rolled onto the powder layer and the latter is compacted at the same time and the metal powder is fired at 800° to 1500° C. in an oxidizing atmosphere. In order to impart to the diaphragms a constant thickness, strength and density, the metal powder is uniformly distributed and applied as regards its bulk volume to the support and the powder layer is moved under a distributing roller rotating opposite to the direction in which the powder is fed.

2 Claims, 1 Drawing Sheet





FIG. 1



FIG. 2

APPARATUS FOR MANUFACTURING  
DIAPHRAGMS

This is a division of application Ser. No. 339,747, filed Apr. 18, 1989, now U.S. Pat. No. 4,961,901.

BACKGROUND OF THE INVENTION

This invention relates to a process of manufacturing diaphragms having a thickness of 0.3 to 3.0 mm and consisting of a wire net, preferably a nickel wire net, which serves as a carrier, and a porous ceramic layer having a thickness of 0.1 to 2.8 mm, which is joined to said wire net, preferably for electrolyses, wherein a layer consisting of a difficulty flowable metal powder, preferably a nickel powder, which consists of irregularly shaped particles, is applied to a support, the wire net is rolled or pressed onto the powder layer and the latter is compacted by 30 to 60% at the same time, and the metal powder is fired in an oxidizing atmosphere at temperatures of 800° to 1500° C. for 1 to 30 minutes, preferably 5 to 15 minutes.

Diaphragms for use in electrolyses should resist elevated temperatures and corrosion. They should not have an electron conductivity of their own and should have an adequate mechanical strength and their thickness should be minimized so that they have a very low resistance to the transport of electric charges in the electrolyte.

In order to accomplish this, EP-B 0 022 252 discloses a diaphragm which has a thickness of 0.3 to 0.7 mm and consists of porous sintered nickel, iron or copper and comprises a skeleton structure which is constituted by a wire net, preferably a nickel wire net, wherein the metal is oxidized at least in part to form metal oxide. To produce such a diaphragm a layer of the metal powder is applied to a wire net having a mesh opening size of 100 to 500  $\mu\text{m}$  in that a paste consisting of the metal powder and a binder or alcohol is spread on or sprayed onto the wire net and is compacted under a pressure of about 200  $\text{kg}/\text{cm}^2$  and is simultaneously bonded to the wire net. The metal powder is subsequently subjected to a reducing sintering treatment at a temperature of 700° to 1000° C. for 10 to 20 minutes and to a succeeding oxidizing treatment at a temperature of 1000° to 1200° C. for up to 3 hours. Said processes can allegedly be carried out to produce diaphragms which have a large surface area and have a strength which is due to the fact that the oxidation is not excessive but a residual metallic structure is obtained. Because the formation of oxide proceeds from the surface throughout the entire body, the electrical resistance is sufficiently high. But it has been found that the diaphragms which have been described hereinbefore, particularly when they have large dimensions, do not have a constant strength, density and thickness throughout the entire body although a constant strength is required for ensuring that the surfaces of the diaphragms will resist an erosion by gas and liquid streams occurring in the cells for an electrolysis of aqueous solutions. A constant density and a constant thickness of the diaphragms are required for ensuring a uniform current density and an optimum purity of gas because a non-uniform current density, i.e., local concentrations of current, may result in local overheating and corrosive attacks, i.e., in a formation of holes in the diaphragms so that oxyhydrogen gas may be formed in the electrolysis of alkaline aqueous solutions.

It has been attempted to manufacture thin diaphragms having a constant strength, density and thickness in that nickel powder is strewn onto a support through a fine-mesh screen which extends over said support at a small distance therefrom, the strewn-on nickel powder layer is compacted by rolling and the nickel wire net is joined to the nickel powder layer at the same time. But said measures will not ensure a uniform distribution of the nickel powder on the support and thus the strength, density and thickness of the resulting diaphragm will not be uniform. Besides, when diaphragms having a large surface area are to be made the screen must be held at a uniform thickness from the support by means of spacers because without a provision of spacers the screen will be deflected by the nickel powder applied to the screen and under the pressure of the doctor blade which is moved over the nickel powder and the distance between the screen and the support will then be non-uniform. Moreover, spacers will form discontinuities in the nickel powder layer and the resulting gaps will strongly adversely affect the separation of the gas and the uniformity of the current flow.

SUMMARY OF THE INVENTION

It is an object of the present invention to improve the process of the kind described first hereinbefore that thin diaphragms having a constant thickness, strength and density and a large surface area can be manufactured by a continuous process.

That object is accomplished in accordance with the invention in that the bulk volume of the metal powder is uniformly distributed and applied to the support in a powder layer and the powder layer is moved under a distributing roller rotating opposite to the direction in which the powder is fed so that a layer of uniform thickness is formed. That measure is required to ensure that the porous ceramic layers which are joined to the wire net will have a uniform thickness and will firmly be bonded to the wire net.

The metal powder is suitably applied to the support at a rate of 25 to 500  $\text{mg}/\text{cm}^2$ .

The metal powder layer which has been moved under the distributing roller suitably has a thickness of 1.0 to 7.0 mm, preferably 3.0 to 5.0 mm.

The object may also be accomplished in that the bulk volume of the metal powder is uniformly distributed and applied to the wire net lying on a support and the powder layer is moved under a distributing roller rotating opposite to the direction in which the powder is fed so that a layer of uniform thickness is formed.

In that case it will be necessary to coat the wire net on both sides wherein the wire net with the powder layer adhering thereto is turned around to lie at the top and a layer consisting of the same metal powder is uniformly distributed and applied and is then moved under a distributing roller rotating opposite to the direction in which the powder is fed, followed by a compaction by rolling.

To provide the wire net with a porous ceramic layer on both sides, a layer of the same metal powder is uniformly distributed and applied as regards its bulk volume to the wire net which has been rolled or pressed onto the first-mentioned powder layer and is moved under a distributing roller rotating opposite to the direction in which the powder is fed, whereby a layer of uniform thickness is formed, and is finally compacted by rolling.

The apparatus for carrying out the process, consists of a star wheel feeder which distributes and applies the pulverulent metal, a distributing roller and a compacting roll, which succeed the star wheel feeder, which compacting roll forces the wire net, which is preferably wound up on a drum, against the metal powder layer so that the openings of the wire net are filled with metal powder.

In a preferred embodiment the star wheel feeder, distributing roller and compacting roll and optionally the drum which cooperates with the compacting roll are combined in a unit which is movable along the support.

To permit a coating of the wire net on both sides within the shortest possible time another star wheel feeder and a distributing roller are associated with the unit consisting of the star wheel feeder, distributing roller and compacting roll. During the forward movement of the unit, the wire net is forced by the compacting roll into the surface of the sintered metal powder layer, which has a constant thickness, and the powder layer is compacted at the same time. During the return movement the metal powder layer which has been applied to the wire net and has a uniform thickness is compacted by the compacting roll. As a result, the irregularly spaced particles of the metal powder are so strongly joined that the resulting composite material can easily be handled. The metal powder particles interlock so strongly that diaphragms which are small in size can be made from said particles without a wire net that serves as a carrier.

The positions of the star wheel feeder and of the outlet opening of the supply bin are so selected that no metal powder can be dispensed when the star wheel feeder is at a standstill. As a result, the rate at which the metal powder is dispensed and the thickness of the layer which is distributed over and applied to the support will depend on the speed of the star wheel feeder. The thickness of the layer of metal powder on the support can also be controlled by the velocity at which the unit consisting of the star wheel feeder, distributing roller and compacting roll is moved.

The composite material can be manufactured in the form of plates or strip and is so flexible that it can be wound up on a drum without difficulty.

The invention is illustrated by way of example on the drawings and will be explained more in detail hereinafter.

#### BRIEF DESCRIPTION OF THE DRAWINGS

FIGS. 1 and 2 are schematic representations of the apparatus for carrying out the process according to the present invention.

#### DESCRIPTION OF THE PREFERRED EMBODIMENT

In accordance with FIGS. 1 and 2, carbonyl nickel powder 2 having a particle size of 2.2 to 2.8  $\mu\text{m}$  is distributed and applied from the hopper-shaped supply bin 1 in batches on the stationary support 4 at a rate of 50  $\text{mg}/\text{cm}^2$  by means of the star wheel feeder 3, which closes the outlet opening of the supply bin 1 and com-

prises coaxially extending trough-shaped cells in a star-like configuration. By the distributing roller 5, which rotates opposite to the direction in which the powder is fed, the carbonyl nickel powder layer 6 is brought to a uniform thickness. The carbonyl nickel powder layer 6 is compacted to a thickness of 0.3 mm by the compacting roll 7, by which the nickel wire net 9, which is wound on the drum 8 and has a wire thickness of 0.125 mm and a mesh opening size of 0.2 mm is rolled onto the carbonyl powder layer at the same time as said net is unwound from the drum 8.

When the nickel wire net 9 has been cut off, carbonyl nickel powder 11 from the supply bin 10 is applied by means of the star wheel feeder 12 to the nickel wire net 9 at a rate of 50  $\text{mg}/\text{cm}^2$ . The powder layer is brought to a uniform thickness by the distributing roller 13, which rotates opposite to the direction in which the powder is fed, and the powder layer is subsequently compacted to a thickness of 0.45 mm by the compacting roll 7.

When the composite material has subsequently been fired in an oxidizing atmosphere at a temperature of 1000° for 15 minutes, the composite material has a constant thickness and constant density throughout its surface area so that an optimum wear resistance, a uniform current distribution and a high purity of the gas will be ensured. The composite material may be profiled before it is fired.

What is claimed is:

1. An apparatus for manufacturing a diaphragm made up of a wire net carrier and a porous ceramic layer joined to the carrier, comprising: a support; first means for applying metal powder onto the support in a first feed direction to form a powder layer thereon, wherein the metal powder is flowable with difficulty and consists of irregularly shaped particles; a first distributing roller rotatable in a direction opposite to the first feed direction; means for moving the applied powder and the support under the distributing roller in the first feed direction while rotating the distribution roller in the direction opposite the first feed direction to impart a uniform thickness to the powder layer; a wire net; means for applying the wire net onto the uniform thickness powder layer and for compacting the uniform thickness powder layer at the same time by 30 to 60% comprising a single compacting roller; second means for applying the metal powder onto the support in a second feed direction to form a second powder layer thereon, a second distributing roller rotatable in a direction opposite to the second feed direction; second means for moving the applied powder and the support under the second distributing roller in the second feed direction while rotating the distribution roller in the direction opposite the second feed direction to impart a uniform thickness to the second powder layer and second means for compacting the uniform thickness second powder layer; and means for firing the compacted powder layers and wire net in an oxidizing atmosphere.
2. The apparatus according to claim 1, including means for making the first and second feed directions opposite to each other.

\* \* \* \* \*